

# UNITED STATES PATENT OFFICE.

CHARLES E. BAKER AND ARTHUR W. BURWELL, OF CLEVELAND, OHIO.

## PROCESS OF TREATING ORES.

No. 841,102.

Specification of Letters Patent.

Patented Jan. 15, 1907.

Application filed July 5, 1904. Renewed July 5, 1906. Serial No. 324,792.

*To all whom it may concern:*

Be it known that we, CHARLES E. BAKER and ARTHUR W. BURWELL, citizens of the United States, residing at Cleveland, in the county of Cuyahoga and State of Ohio, have invented certain new and useful Improvements in Processes of Treating Ores, of which the following is a specification.

This invention is a process for the treatment of ores which contain the sulfids of such metals as yield fusible chlorids.

The process will be particularly described as applied to the separation of lead and zinc from their sulfid ores; but the invention is not limited to the recovery of these particular metals.

The dry ore containing the sulfids of lead or zinc is finely pulverized and brought into contact with sulfur chlorid, ( $S_2Cl_2$ ). The pulverized ore is preferably exposed in a revolving drum or other suitable reaction vessel to the vapor of sulfur chlorid, said vapor being either introduced from without or being produced in the reaction vessel by applying heat thereto. In either case the ore is preferably heated to hasten the reaction. The sulfur of the ore is replaced by the chlorid of the sulfur chlorid with separation of sulfur from both of the reacting bodies in accordance with the equation



in which M represents a metal, as lead or zinc, whose chlorid is fusible.

We do not limit ourselves to any particular temperature for carrying out the reaction; but we prefer to heat the ore above the fusing-point of the chlorid of the metal or metals to be recovered. The separated sulfur may be skinned or run from the molten chlorid, or if the temperature be above the vaporizing-point of sulfur it may be distilled and recovered in any suitable condensing apparatus.

We prefer to electrolyze the metallic

chlorid for the recovery of the metal. In 45 such case the anode is preferably of graphite, and the cathode may consist of a molten body of the metal to be recovered. The chlorin separated at the anode may be used for producing sulfur chlorid to be used in the 50 continuation of the process or may be otherwise utilized as desired.

We claim—

1. The process which consists in subjecting pulverulent sulfid ores of metals forming 55 fusible chlorids to the action of sulfur chlorid, thereby producing the chlorid of the metal, fusing said chlorid and recovering the metal, substantially as described.

2. The process which consists in subjecting 60 pulverulent sulfid ores of metals forming fusible chlorids to the action of sulfur chlorid, thereby producing the chlorid of the metal, fusing said chlorid and recovering the metal by electrolyzing the fused chlorid, substan- 65 tially as described.

3. The process which consists in subjecting pulverulent sulfid ores of metals forming fusible chlorids at a temperature above the fusing-point of the chlorid to the action of 70 sulfur chlorid, thereby producing the chlorid of the metal and recovering the metal from the fused chlorid, substantially as described.

4. The process which consists in subjecting pulverulent sulfid ores of metals forming 75 fusible chlorids at a temperature above the fusing-point of the chlorid to the action of sulfur chlorid, thereby producing the chlorid of the metal and recovering the metal by electrolyzing the fused chlorid, substantially 80 as described.

In testimony whereof we affix our signatures in presence of two witnesses.

CHARLES E. BAKER.

ARTHUR W. BURWELL.

Witnesses:

FRANK N. SEALAND,

CARL RUSSELL FOSTER.